

W. D. RICE,  
PROCESS FOR MAKING SHRAPNEL SHELLS,  
APPLICATION FILED SEPT. 22, 1917.

1,303,727.

Patented May 13, 1919.

A

Fig. 1.



A

Fig. 2.



Fig. 3.



Fig. 4.



Fig. 5.



Inventor

William D. Rice  
By *Paul Boggs & Co*  
Attorneys

# UNITED STATES PATENT OFFICE.

WILLIAM D. RICE, OF CONNEAUT, OHIO.

## PROCESS FOR MAKING SHRAPNEL-SHELLS.

1,303,727.

Specification of Letters Patent. Patented May 13, 1919.

Application filed September 22, 1917. Serial No. 192,703.

*To all whom it may concern:*

Be it known that I, WILLIAM D. RICE, a citizen of the United States, residing at Conneaut, in the county of Ashtabula and State of Ohio, have invented certain new and useful Improvements in Processes for Making Shrapnel-Shells, of which the following is a specification.

My invention relates to an improvement in the process for making shrapnel shells.

The object is to provide and construct a shell of a frangible nature, which will be so constructed that it will burst upon explosion into innumerable fragments, due to a difference in the strength of its walls at certain areas.

It therefore consists in a shell of the character specified, and in a method of construction, in which there are a series of operations, to wit:—the casting of a hollow shell of steel, which might be termed commercial cast steel, with walls of unequal thickness; a re-heating of the shell; compressing the shell; carburizing the shell; and finally machining and reducing to a perfect surface, whereby parts are removed, thereby leaving a shell made up of hard and soft areas.

In the accompanying drawings:—

Figure 1 is a longitudinal sectional view before machining;

Fig. 2 is a similar view after machining;

Fig. 3 is a transverse section through Fig. 1;

Fig. 4 is a transverse section through Fig. 2;

Fig. 5 is a view showing the application of the invention to both surfaces of the shell.

A, is a cast shell, which may have grooves cast in the internal or external surface, or both, as shown in Figs. 1 and 5, thus leaving raised areas which may be square, diamond-shape, or any other form.

After casting, the shell is placed in an oven or retort and heated to a temperature of approximately 1400° F. for the purpose of giving it uniformity of hardness.

The shell is then removed from the oven or retort, after having reached approximately the degree of temperature specified, whereupon it is subjected to a longitudinal pressure for the purpose of eliminating porous places which might be caused by the separation of gases while cooling. There are several reasons for the longitudinal pressing of the shell, one of the essential of

which is the making of the grain in the thinner places of the shell more dense than in the thicker areas.

It is a well-known fact that when steel cools, the thicker portions have a tendency to pull away from the thinner portions, causing a slight deterioration of the grain in the thinner places, which is known among those engaged in casting steel as "shrinkage cracks" which have a tendency to weaken the areas where this condition exists, and nothing but re-melting could ever give these places the same consistency as the thicker places of the casting.

After the shell is thus cast, re-heated and compressed, it is carburized in any approved manner, and with any well-known material, as for instance by the use of granulated bone such as ground bone or any other carbonaceous material. Either or both surfaces may be carburized, but it is my intention to carburize only the grooved surface, whether that be the interior or exterior or both surfaces of the shell.

An approved method of carburizing would be to place the shell in cast-iron boxes, lead crucibles, or whatever containers the manufacturer deems desirable, in which the shell is packed loosely with granulated bone such as ground bone or other carbonaceous material. To harden the shell, it is subjected to a quenching process, and the part of the shell that has been combined with the carbon will harden to a greater degree than the raised portions, and the quenching process should not be carried sufficiently far to make the shell too brittle for use. Either water, oil, or air can be used for quenching. This is the last process to which the shell is subjected.

There is a final machining which takes place which results in removing the thickened portions left by the grooves in casting, thus making the shell of uniform thickness instead of irregular thickness as at the beginning; and it is due to this final machining, which removes or reduces these thickened areas, and, consequently, the carburized or hardened surface of these areas, that the completed shell is made up of hard and soft areas, which results in its fracture, upon an explosion taking place, in a maximum number of parts.

By means of this improved process, the completed shell will have a hard, brittle and

friable surface, and the harder and more friable places will be in the lines between the original raised areas, which, in the end, have been machined off. As previously 5 stated, this is due to the fact that the thinnest part of the shell will have the closest grain, thus being more susceptible to carburizing, and hence will be more brittle than the parts under the raised portions which 10 have been re-heated and machined off, and the result will be that the shell will break in practically as many pieces as there were originally thickened areas.

The temperature of annealing of steel 15 castings depends entirely upon the chemical composition. For instance, for an ordinary steel casting of about .30 carbon, with .60 manganese, .20 silicon, .05 phosphorus, and .105 sulfur, the annealing temperature would 20 be approximately 1575 to 1600. This would be lowered for a higher carbon and raised for a lower carbon. It would likewise be raised for a lower manganese and lowered for a higher manganese, but the figures 25 which I have given are approximately standard for the ordinary steel casting.

I do not desire to be limited to any particular method of casting, re-heating, com-

pressing, or carburizing, but my invention comprises a process combining these steps.

I claim:

1. An improved method of constructing shells, which consists in casting a shell of steel with a body of varying or irregular thickness, re-heating the shell to the required degree, subjecting it to compression, carburizing the irregular surface to a suitable depth, and finally machining or otherwise removing the irregular surface to give it uniformity, thereby removing the thickened areas and the portions thereof which are hardened, and leaving the intervening hardened areas.

2. An improved method of constructing shells, which consists in casting a shell of steel with a body of varying or irregular thickness, re-heating the shell to the required degree, subjecting it to compression, case hardening the irregular surface to a suitable depth, then machining or otherwise removing the irregular surface to give it uniformity, then re-heating and finally quenching.

In testimony whereof I affix my signature.

WILLIAM D. RICE.